

## UNITED STATES PATENT OFFICE

2,252,675

STABILIZED HYDROCARBON COMPOSITION  
AND STABILIZING AGENT THEREFOR

Carl F. Prutton, Cleveland Heights, Albert K. Smith, Shaker Heights, and Delton R. Frey, East Cleveland, Ohio, assignors to The Lubri-Zol Corporation, Wickliffe, Ohio, a corporation of Ohio

No Drawing. Application March 6, 1939,  
Serial No. 260,220

24 Claims. (Cl. 252—53)

This invention relates, as indicated, to the stabilization of hydrocarbon compositions. The term "hydrocarbon compositions" as used herein, is intended to include liquid compositions which are essentially derivatives of petroleum, naturally occurring oils of the type represented by animal, vegetable and marine oils and derivatives of the same.

More specifically, this invention relates to the stabilization of hydrocarbon compositions, such as lubricants which are usually essentially mineral oil. This invention also is applicable to the stabilization of lighter fractions of petroleum such as are used as fuels.

Certain subject matter disclosed but not claimed herein is disclosed and claimed in co-pending applications Serial No. 260,221, filed March 6, 1939, and Serial No. 395,234, filed May 26, 1941.

It is well known that liquid hydrocarbon compositions of the character above identified are subject to deterioration as by oxidation and polymerization, for example but not by way of limitation, during storage and handling and are also subject to deterioration which proceeds at a more rapid rate during use of these compositions.

For example, the various oils mentioned above and the lighter fractions used as fuels have a tendency on storage to oxidize, polymerize, or otherwise deteriorate to form gums and the like; and when such compositions are used, particularly under conditions of high temperature, deterioration proceeds at a more rapid rate to the production of gums, sludges and other oxidation and/or polymerization products. This deterioration is manifested by discoloration of the liquid hydrocarbon body; the generation within the body of flocculent material; the precipitation from the body of the more serious types of deterioration products, such as sludge, and the deposit of varnish or shellac-like deposits on metallic surfaces with which the compositions come in contact during use.

Liquid hydrocarbon compositions, such as refined mineral oil, when employed for use as lubricants in internal combustion engines whether of the ignition or Diesel type are generally subject to the various conditions above named which tend to cause deterioration of such oil composition. Oxidation and/or sludging of liquid hydrocarbon compositions employed as lubricants in such engines is usually accelerated by the relatively high temperatures to which such compositions are subjected. This is particularly true in engines of the Diesel type in which the op-

erating temperatures are generally somewhat higher than those in the so-called ignition type.

It is a principal object of our invention, therefore, to provide for the stabilization of compositions of the character defined in order to reduce the tendency of the same to decompose particularly in the manner indicated.

It will also be observed that the addition agents employed for the prescribed purpose are in themselves new compositions of matter.

Other objects of our invention will appear as the description proceeds.

Broadly stated, this invention comprises the improvement of the properties of liquid hydrocarbon compositions of the character previously identified, and particularly the stabilization of such compositions under conditions of use, by the inclusion therein of a minor proportion of the product resulting from the reaction of a hydroxy ester or an organic hydroxy-acid with a reagent which comprises phosphorus in tri-valent form and a halogen. It also comprises the similar use of certain derivatives of these reaction products.

As hereinafter more fully explained, the stabilization of certain types of liquid hydrocarbon compositions and especially when the same are used for certain specific purposes, may be effected by the inclusion therein of certain derivatives of the aforesaid reaction product or products or portions thereof, which derivatives may be prepared, for example, by halogenation and/or treatment with an alkali or other base to form a salt, or ester-salt.

As previously stated, our invention contemplates the use, as stabilizing agents, of the products resulting from a specified reaction. We therefore list below specific examples of the two classes of reactants which may be employed in the preparation of the product which we employ as the stabilizing addition agent.

*The phosphorus and halogen containing reactants*

As indicated above, any material which contains phosphorus in tri-valent form and a halogen, which material will react with a hydroxy ester, may be employed in the preparation of an addition agent. Of these phosphorus and halogen containing reactants,  $PCl_3$  will be found to be particularly useful and productive of suitable addition agents. Other reactants of this class are as follows:

Phosphorus tri-bromide,  $PBr_3$

Phosphorus tri-iodide,  $PI_3$

Phosphorous oxy-chloride,  $POCl$

Phosphorous sulpho-chloride,  $PSCl$

Halogen derivatives of phosphine and organic substituted phosphines, e. g.

Phosphenyl chloride,  $(C_6H_5)PCl_2$

Compounds of the classes:

(a)  $RPCl_2$  and  $RR'PCl_2$ , and (b)  $ROPCl_2$  and  $(RO)(R'O)PCl$  in which R and R' are organic radicles such as:

Aromatic, e. g.

Phenyl

Cyclohexyl phenyl

Alkylated phenyl

Aliphatic, e. g.

Lauryl

Cetyl

Cycloaliphatic, e. g.

Cyclopentyl

Cyclohexyl

*The hydroxy esters*

The esters which are suitable for use as one of the components of the reaction with phosphorus and halogen containing reactants in the preparation of the stabilizing addition agent of our invention may, for example, be any of the esters produced by reacting any of the alcohols, and preferably any of the mono- or di-hydroxy low molecular weight alcohols, such as any of the following:

Methyl alcohol

Ethyl alcohol

Propyl alcohol

Butyl alcohol

Ethylene glycol

Propylene glycol

Trimethylene glycol

Cyclohexanol

Benzyl alcohol

Furfuryl alcohol

with any organic hydroxy-acid, and preferably with any saturated monobasic or polybasic hydroxy-fatty acid such as any of the following:

(1) Monobasic acids:

(a) Monohydroxy: e. g.

Glycolic acid

Lactic acid

Hydracrylic acid

Hydroxylbutyric acids

(b) Polyhydroxy: e. g.

Glyceric acid

Dihydroxy palmitic acid

(2) Polybasic acid

(a) Monohydroxy: e. g.

Tartaric acid

Malic acid

Citramalic acid

Citric acid

(b) Polyhydroxy: e. g.

Tartaric

Trihydroxy glutaric acid

In general, the esters of the low molecular weight hydroxy-fatty acids are preferred.

We have found the methyl esters to be preferable for our purpose in most cases.

The following are illustrative of specific embodiments of our invention:

A material, which for purposes of convenience in referring to the same herein we shall designate as P. M. L., is prepared by the reaction of methyl lactate with  $PCl_3$ . The relative proportions of methyl lactate and  $PCl_3$  used in the preparation of P. M. L. are given in the following table, as well as the properties of the end product.

| <i>Example I (P. M. L.)</i> |                            |
|-----------------------------|----------------------------|
| 5                           | Methyl lactate             |
|                             | 104 parts by weight        |
|                             | $PCl_3$                    |
|                             | 45 parts by weight         |
|                             | Weight of product          |
|                             | 74.5                       |
| 10                          | Weight of material removed |
|                             | by distillation            |
|                             | 31.8                       |
|                             | Yield                      |
|                             | 65%                        |
|                             | Average mol. wt.           |
|                             | 312                        |
|                             | Boiling point              |
|                             | 230° C.                    |
|                             | Melting point              |
|                             | Liquid at room temperature |
|                             | Sp. gr. at 20° C.          |
|                             | 1.252                      |
|                             | Ref. index at 26° C.       |
|                             | 1.4365                     |
| 15                          | Color                      |
|                             | Light yellow               |
|                             | Phosphorus                 |
|                             | 10.9%                      |
|                             | Chlorine                   |
|                             | 1.12%                      |
|                             | Acid No.                   |
|                             | 415                        |

Soluble to extent of about 1% in Penna 150 (S. U. S. at 100° F.) neutral.

Completely miscible with water and ethyl alcohol.

The methyl lactate is placed in a reaction vessel equipped with an agitator and reflux condenser. The vessel and agitator are preferably 25 of glass or enamel. The  $PCl_3$  is added slowly and the temperature of the reactants maintained below 60° C. during the addition of the  $PCl_3$ . The mixture is stirred continuously during the addition of the  $PCl_3$ . The temperature of the 30 reactants may be controlled by the rate of the addition of the  $PCl_3$ . After the addition of the  $PCl_3$  is complete, the mixture is agitated until the temperature begins to decrease, indicating that the  $PCl_3$  has reacted to some extent with the methyl lactate. The slow addition of  $PCl_3$  accompanied by stirring until a decrease in temperature is noted insures against loss of  $PCl_3$  whose boiling point is 76° C. and also gives a higher yield than when these precautions are not taken. After the temperature of the reactants has begun to drop, heat is applied and the temperature of the reactants is raised to 120° C. This temperature is maintained for 3 hours. A slight reaction is apparent until the mixture has 45 been heated at 120° C. for about 2 hours and 45 minutes. The mixture is stirred continuously all during the time of adding the  $PCl_3$  and maintaining at 120° C.

After completion of the reaction between the 50 methyl lactate and  $PCl_3$ , i. e., after the mixture has been maintained at a temperature of 120° C. for about 3 hours, the end product may either be used as such as a stabilizing addition agent for liquid hydrocarbon compositions or the end 55 product may be distilled at atmospheric pressure and all of the material which distills over at 130° C. or less may be discarded. Whether the end product as produced or the refined end product derived by removal of the more volatile products 60 is used, depends largely upon the use for which the ultimate composition containing the stabilizing addition agent is designed. In general, the less volatile part of the reaction product, or that part which contains combined phosphorus, 65 is preferred for our purpose.

We believe the reaction produces two general types of compounds:

(a) Chlorine-containing compounds, for example the type in which chlorine has been substituted for the hydroxyl group of the hydroxy-ester; and

(b) Phosphorus-containing compounds, for example the type in which the hydroxyl group has lost hydrogen (which forms HCl with chlo-

rine removed from the  $\text{PCl}_3$ ) so that the oxygen of the hydroxyl group becomes attached to a phosphorus atom.

(the refined material) to several different representative commercial oils, and oils treated with other addition agents.

| Example No. | Composition                |                       |                 |                |                  | Oxidation test   |            |                              |            |                            |                   |                   | Corrosion test (lead-bronze) |  |
|-------------|----------------------------|-----------------------|-----------------|----------------|------------------|------------------|------------|------------------------------|------------|----------------------------|-------------------|-------------------|------------------------------|--|
|             | Hexa-chlor-di-phenyl-oxide | Ortho-dichlor-benzene | Methyl stearate | Butyl stearate | Percent P. M. L. | Conradson carbon |            | Viscosity S. U. S. @ 210° F. |            |                            | Naphtha Insoluble |                   |                              |  |
|             |                            |                       |                 |                |                  | Original         | @ 48 hours | Original                     | @ 48 hours | Percent viscosity increase | Hours for 10 mg.  | Hours for 100 mg. | Mg. @ 48 hours               |  |

NAPHTHENIC BASE ACID TREATED S. A. E. 30 DIESEL OIL

|    |            |  |  |  |  |     |      |      |      |      |      |      |     |      |      |
|----|------------|--|--|--|--|-----|------|------|------|------|------|------|-----|------|------|
| 1. | Un-treated |  |  |  |  | .08 | 2.15 | 54.9 | 70.9 | 29.2 | 14   | 34   | 249 | -.24 |      |
| 2. |            |  |  |  |  | .03 | .08  | .88  | 54.7 | 60.4 | 10.4 | 28.5 | 8   | 20   | -.26 |

MID-CONTINENT S. A. E. 30 MOTOR OIL

|    |            |     |     |     |  |     |      |      |      |      |      |      |     |      |      |
|----|------------|-----|-----|-----|--|-----|------|------|------|------|------|------|-----|------|------|
| 3. | Un-treated |     |     |     |  | .32 | 1.67 | 63.1 | 74.4 | 17.9 | 13.5 | 44   | 121 | -.18 |      |
| 4. |            |     |     |     |  | .03 | .43  | 1.27 | 63.9 | 69.0 | 7.1  | 32.5 | 8   | 42   | -.02 |
| 5. |            |     |     |     |  | .06 | .43  | 1.61 | 67.1 | 71.0 | 5.9  | 28.5 | 8   | 56   | -.06 |
| 6. | .30        | .30 |     |     |  | .08 | 1.82 | 63.6 | 73.1 | 16.0 | 17.0 | 46   | 111 | -.51 |      |
| 7. | .30        | .30 |     |     |  | .06 | .57  | 1.28 | 63.1 | 68.3 | 8.2  | 37.0 | 8   | 34   | -.12 |
| 8. | .60        | .50 | .25 | .25 |  | .41 | 2.05 | 61.6 | 72.2 | 17.2 | 13.0 | 45   | 118 | -.02 |      |
| 9. | .50        | .50 | .25 | .25 |  | .03 | .78  | 1.18 | 62.1 | 69.0 | 11.1 | 35.0 | 8   | 40   | -.06 |

COMMERCIAL S. A. E. 10 MOTOR OIL HAVING A V. I. OF 67

|     |            |     |  |  |  |     |      |      |      |      |     |      |      |      |      |
|-----|------------|-----|--|--|--|-----|------|------|------|------|-----|------|------|------|------|
| 10. | Un-treated |     |  |  |  | .08 | 2.81 | 42.8 | 48.2 | 12.6 | 7.0 | 24.5 | 375  | -.22 |      |
| 11. |            |     |  |  |  | .03 | .04  | 1.20 | 42.7 | 45.5 | 6.5 | 10.5 | 41.5 | 100  | -.07 |
| 12. | .30        | .30 |  |  |  | .03 | .12  | 42.9 | 48.9 | 14.0 | 5.0 | 20.0 | 414  | -.23 |      |
| 13. | .30        | .30 |  |  |  | .06 | .01  | 1.54 | 42.8 | 45.9 | 7.3 | 19.0 | 40.0 | 180  | -.09 |

PENNSYLVANIA S. A. E. 40 MOTOR OIL

|     |            |     |     |     |  |      |      |      |       |       |      |   |     |      |
|-----|------------|-----|-----|-----|--|------|------|------|-------|-------|------|---|-----|------|
| 14. | Un-treated |     |     |     |  | 1.25 | 3.52 | 82.7 | 104.0 | 26.3  | 8    | 8 | 5   | -.08 |
| 15. |            |     |     |     |  | .03  | 1.46 | 2.51 | 83.0  | 95.7  | 15.3 | 8 | 2   | -.46 |
| 16. |            |     |     |     |  | .06  | 1.51 | 2.51 | 83.0  | 95.8  | 15.4 | 8 | 2   | -.28 |
| 17. | .30        | .30 |     |     |  | .08  | 1.67 | 3.54 | 82.3  | 104.0 | 26.5 | 8 | 3   | -.38 |
| 18. | .30        | .30 |     |     |  | .06  | 1.24 | 2.32 | 81.4  | 94.0  | 15.5 | 8 | 0.7 | -.09 |
| 19. | .50        | .50 | .25 | .25 |  | .03  | 1.19 | 2.80 | 79.6  | 98.9  | 24.2 | 8 | 6   | -.35 |
| 20. | .50        | .50 | .25 | .25 |  | .03  | 1.40 | 2.60 | 81.9  | 94.9  | 15.8 | 8 | 0.6 | -.10 |

PENNSYLVANIA S. A. E. 10 MOTOR OIL

|     |            |     |     |     |  |     |     |      |      |      |      |        |    |       |
|-----|------------|-----|-----|-----|--|-----|-----|------|------|------|------|--------|----|-------|
| 21. | Un-treated |     |     |     |  | .23 | .94 | 47.1 | 49.8 | 5.7  | 25.0 | 8      | 45 | -1.15 |
| 22. |            |     |     |     |  | .03 | .16 | .45  | 46.5 | 47.8 | 2.8  | (64.0) | 2  | -.84  |
| 23. |            |     |     |     |  | .06 | .30 | .50  | 46.3 | 47.6 | 2.8  | 8      | 3  | -.31  |
| 24. | .30        | .30 |     |     |  | .06 | .15 | 1.40 | 46.3 | 50.6 | 9.8  | 22.0   | 65 | -1.40 |
| 25. | .30        | .30 |     |     |  | .06 | .20 | .75  | 46.9 | 48.7 | 2.8  | 38.5   | 17 | -.05  |
| 26. | .50        | .50 | .25 | .25 |  | .03 | .21 | 1.19 | 46.5 | 50.0 | 7.5  | 23.0   | 85 | -1.40 |
| 27. | .50        | .50 | .25 | .25 |  | .03 | .21 | .81  | 47.5 | 49.1 | 2.8  | 30.0   | 19 | -.17  |
| 28. | .75        | .75 | .25 | .25 |  | .03 | .13 | 1.13 | 47.3 | 50.8 | 7.4  | 21.0   | 45 | -1.15 |
| 29. | .75        | .75 |     |     |  | .08 | .19 | .87  | 46.6 | 49.0 | 5.1  | 34.0   | 39 | -.07  |

\* Methylidichlorstearate.

a = did not produce 10 mg. in 48 hours.

b = did not produce 100 mg. in 48 hours.

For example in the reaction of methyl lactate with  $\text{PCl}_3$ , part a would be principally the methyl ester of chlor propionic acid and part b principally esters of phosphorous acid such as  $\text{P}(\text{OC}_2\text{H}_5\text{COOCH}_3)_3$  and  $\text{POH}(\text{OC}_2\text{H}_5\text{COOCH}_3)_2$ . It appears that the constituents of the reaction product described as part b are responsible for the stabilizing effect when the product is used in accordance with our invention. However, for most purposes, part a is not deleterious, and for some purposes may even be advantageously included. Part a is in general more volatile than part b and may therefore be easily separated from the latter by distillation at atmospheric or subatmospheric pressure.

The specific properties given in the table captioned "Example No. I" are those for the refined material.

The following table gives the results obtained by the addition of minor amounts of P. M. L.

The determinations which appear in the foregoing table, such as, for example, Conradson carbon, viscosity determinations, and naphtha insoluble, were determined on samples prepared by an oxidation test procedure which is, in every respect, similar to that prescribed by the Standard of Indiana oxidation test, excepting that a piece of iron wire is submerged in the oil during the test.

The data given in the column headed "Corrosion" has been determined in accordance with the standard Shell corrosion test using lead bronze as the metal.

A series of tests substantially duplicating those given in the foregoing table but employing the unrefined P. M. L., i. e., the product immediately resulting from the reaction between methyl lactate and  $\text{PCl}_3$ , and without distilling off any of the end product as hereinbefore specified, were run with substantially the same results as those

given in the foregoing table. It would appear, therefore, that it is not necessary for most uses to refine the P. M. L. before it is used as an addition agent.

Another product which we shall hereinafter, for convenience, refer to as P. B. T. was made by reacting dibutyl tartrate with  $\text{PCl}_3$  under substantially the conditions previously specified for the manufacture of P. M. L., and the following is a table giving the proportions by weight of the reactants used and the properties of the end product.

*Example II (P. B. T.)*

|                            |                            |
|----------------------------|----------------------------|
| Dibutyl                    | 65 parts by weight         |
| $\text{PCl}_3$             | 11.6 parts by weight       |
| Weight of product          | 60                         |
| Weight of refined material | 55.5                       |
| Yield                      | 90%                        |
| Boiling point              | 235° C.-245° C.            |
| Melting point              | Liquid at room temperature |

Tests on oils similar to those given above in connection with the study of the properties of P. M. L. were run using P. B. T., and the latter was found to be substantially as effective as P. M. L.

Another material which we shall hereinafter, for convenience, refer to as P. M. C., was made by the reaction of trimethyl citrate with  $\text{PCl}_3$ . The proportions of reactants used and the properties of the end product are given in the following table:

*Example III (P. M. C.)*

|                            |                     |
|----------------------------|---------------------|
| Trimethyl citrate          | 500 parts by weight |
| $\text{PCl}_3$             | 75 parts by weight  |
| Weight of product          | 480                 |
| Weight of refined material | 465                 |
| Yield                      | 92%                 |
| Melting point              | 80°-100° C.         |

Tests on this material in oil to determine its effect similar to those tests previously given in connection with the study of the effect of P. M. L. were run and show that P. M. C. was similar to P. M. L., i.e., effective to retard deterioration of the oils. P. M. C. has a tendency to be corrosive with respect at least to certain of the more sensitive metals, and, therefore, when such metals are encountered it would be advisable to employ minor amounts of corrosion inhibitors, such as the alkyl and aryl phosphites, along with the P. M. C.

Our invention also contemplates the employment as a stabilizing agent of the reaction products which may be prepared by either of the following methods, viz:

(a) Reacting a reagent, which comprises phosphorus in tri-valent form and halogen, with a mixture of hydroxy esters, a mixture of organic hydroxy acids or a mixture of one or more hydroxy esters with one or more organic hydroxy acids.

(b) Reacting a reagent, which comprises phosphorus in tri-valent form and halogen, with one or two molecules of a hydroxy ester or an organic hydroxy acid per molecule of reagent and then completing the reaction with another reactant of the class consisting of hydroxy esters and organic hydroxy acids different from that which was initially employed.

The reaction products thus prepared are especially desirable for use for certain purposes on account of their complexity.

Very small amounts of our addition agents above identified, are effective, in most cases less than one percent, and usually a fraction of 1%, e. g. from about 0.001 to about 0.2% will be found most useful. For use in mineral lubricating oil (e. g. a motor oil for automobile, aviation, or Diesel engines) amounts from about 0.01% to about 0.1% are suitable, and usually about 0.03% is preferable.

As indicated above, our invention also contemplates the use of oil-soluble derivatives of the above-identified reaction products. (In this connection we are more particularly concerned with the phosphorus-containing constituents of such reaction products.) Such derivatives include the oil-soluble salts and ester-salts, which may be produced by substituting a metal or basic radicle for one or more of the alcohol-derived radicles of the ester. This is conveniently accomplished by partly or completely saponifying the reaction product with an alkali (e. g. sodium, potassium, ammonium, or substituted ammonium, hydroxides) in aqueous solution. Ester-salts may be formed by the partial saponification of esters of polybasic acids, e. g. the phosphorus-containing reaction product of  $\text{PCl}_3$  with dibutyltartrate may be partly saponified with caustic soda to form the corresponding butyl-sodium ester-salt. Similar salts and ester-salts of metals other than the alkali metals may be formed directly by reacting the ester with the metallic base, or more readily by double-decomposition of the alkali salt (or ester-salt) with a salt of the other metal.

As above indicated, our addition agents are suitable for the purpose of stabilizing liquid hydrocarbons generally, among which may be mentioned refined mineral oils of the character generally employed as lubricants, lighter fractions and cuts such as are employed as fuels in Diesel type engines and even lighter fractions and cuts which are commonly identified as gasoline. Other oils such as hydrogenated oils and volatilized oils may be similarly stabilized by the inclusion therein of the above-mentioned addition agents.

The liquid hydrocarbon compositions which may be stabilized by the use of the addition agents hereinbefore specified need not be pure hydrocarbons but may contain other addition agents such as extreme pressure addition agents on the order of halogen, phosphorus and/or sulfur compounds, as well as corrosion inhibitors, such as phosphorus compounds, etc. and other additions commonly employed, such as pour-point depressors and the like.

When a lighter fraction, as above indicated, is stabilized the addition agents commonly employed in such lighter fractions may also be present; as for example, the various "dopes" commonly employed in Diesel fuels, and anti-knock compounds commonly employed in gasolines such as tetra-ethyl lead, iron carbonyl, etc.

In general, the addition agents of this invention will not be found incompatible with commonly employed antioxidants such as are used in gasolines and the like.

There may, however, be certain of these other addition agents which might be found incom-

patible with the addition agents of the present invention and in such cases, of course, the incompatible addition agent, whatever it may be, should be omitted, since it will usually be found that a compatible addition agent for the desired purpose will be available among others of those available.

Among the other addition agents with which the compounds of the present invention may be employed to advantage, as above stated, are the extreme pressure addition agents, such as the halogen, phosphorus and/or sulfur-containing compounds.

In general we have found that the addition agents of the present invention do not detrimentally affect the extreme pressure characteristics of a mineral lubricating oil, for example, which characteristics are the result of the presence therein of the extreme pressure addition agents above named. Moreover, where the addition agents of the present invention have been tested in lubricating compositions which also contain certain other addition agents, the extreme pressure characteristics of the resultant composition has been somewhat improved and such improvement has been traceable to the presence therein of the compounds of the present invention.

Throughout the foregoing specification and in the appended claims, reference is made to "oil-soluble" and by such term, as used herein, it is intended to indicate the ability of the addition agent to form not only true solutions with the oil to which the same are added, but also the ability to form therewith any form of substantially permanently homogeneous composition.

With certain of the more difficultly soluble addition agents to which this application relates, it may be advantageous to employ a mutual solvent as one means for increasing the "oil-solubility" of the addition agents and to also incorporate the addition agents in the oil base by special homogenizing apparatus, such as for example, that described in Cornell Patent No. 2,042,880.

Irrespective, therefore, of the manner in which the addition agent is incorporated in the liquid hydrocarbon, either as a true solution or a permanently stable homogeneous mixture, these various expedients are intended to be included by the term "oil-soluble," as employed herein. Furthermore, those addition agents which are not "oil-soluble" to any extent and which may not be incorporated in such a way as to effect any improvement in the oil, will obviously be excluded by the term "oil-soluble," as employed in the specification and in the claims.

In general, the addition agents prepared in the manner specified will be sufficiently non-volatile so as to find usefulness for the purposes specified. In cases, however, where high temperatures are encountered, it will be best to select those which will neither substantially evaporate from the liquid hydrocarbon and those which will not be decomposed by the temperatures which the composition encounters in use. These limiting factors which must obviously be observed in the selection of any addition agent for use in liquid hydrocarbons are, therefore, intended to be included by the definition "stable" wherever used herein.

In the foregoing specification, reference has been made to optimum percentages within which the addition agents may be employed. It is with-

5 in the contemplation of our invention, however, to admix the addition agents with the specified liquid hydrocarbons up to the limit of their solubility. This may be done advantageously in making concentrates, for example, to be blended with bodies of the same or different liquid hydrocarbons. In other words, the concentrate formed by dissolving the addition agent in a particular hydrocarbon may be dissolved or admixed with another hydrocarbon. In this way advantages of increased solubility may be realized as well as other advantages flowing from the combination of the constituents named. For example, it is within the contemplation of our invention to add to a light hydrocarbon fraction such as gasoline or Diesel fuel, minor amounts of a heavier liquid hydrocarbon such as refined mineral lubricating oil to which has been added a minor amount of the addition agents which characterize the present invention. Such combination, i. e., a major proportion of gasoline to which has been added a minor amount of a mineral oil of lubricating viscosity for internal combustion engine use, along with a minor amount of the addition agents which characterize the present invention, produces a fuel for internal combustion engines which is particularly desirable for use on account of the nature of the deposits left by the fuel in the combustion chamber, as well as the general performance of the fuel.

For proper results, when the compounded relatively heavier liquid hydrocarbon is essentially mineral oil having a viscosity of from about 50 to about 250 seconds Saybolt Universal at 100° F., such composition should be added to the usually lighter hydrocarbon fuel of the type boiling within the gasoline range in quantities varying from .05% to 1.50% by volume. The amount of compounded heavier hydrocarbon added to the lighter hydrocarbon fuel for optimum results will be found to be in the vicinity of .30%, i. e., in the range of from about 0.15% to 0.60%.

It will be observed that the addition agents mentioned above may be generally classified as follows:



where  $R'$ ,  $R^3$  and  $R^5$  are organic radicles; and  $R^2$ ,  $R^4$  and  $R^6$  are organic radicles, hydrogen, a metal, or a metallic radicle.



where  $R'$ ,  $R^3$ ,  $R^5$  and  $R^8$  are organic radicles and  $R^2$  and  $R^4$  are organic radicles, hydrogen, a metal, or a metallic radicle.



where  $R'$ ,  $R^3$ ,  $R^5$  and  $R^6$  are organic radicles and  $R^2$  and  $R^4$  are organic radicles, hydrogen, a metal, or a metallic radicle.

Other modes of applying the principle of our invention may be employed instead of the one explained, change being made as regards the materials employed, provided the ingredients stated by any of the following claims or the equivalent of such stated ingredients be employed.

We, therefore, particularly point out and distinctly claim as our invention:

1. A lubricating composition comprising a major proportion of mineral oil, the properties of which affecting its use as a lubricant are improved by the inclusion therein of a minor proportion of an oil-soluble product resulting from the reaction of a hydroxy-ester with a phosphorus and halogen containing compound of the type in which the phosphorus is present in the tri-valent form.

2. A lubricating composition comprising a major proportion of mineral oil, the properties of which affecting its use as a lubricant in the crank-case of an internal combustion engine are improved by the inclusion therein of a minor proportion of the phosphorus-containing product resulting from the reaction of an ester of an organic hydroxy-acid with a phosphorus and halogen containing compound of the type in which the phosphorus is present in tri-valent form.

3. A lubricating composition comprising a major proportion of mineral oil, the properties of which affecting its use as a lubricant in the crank-case of an internal combustion engine are improved by the inclusion therein of a minor proportion of the phosphorus-containing product resulting from the reaction of  $PCl_3$  with a di-butyl tartrate.

4. A lubricating composition comprising a major proportion of mineral oil, the properties of which affecting its use as a lubricant in the crank-case of an internal combustion engine are improved by the inclusion therein of a minor proportion of the phosphorus-containing product resulting from the reaction of  $PCl_3$  with trimethyl citrate.

5. A lubricating composition comprising a major proportion of lubricating oil, the resistance of which to the formation of deleterious products when exposed to high temperatures under conditions of use is improved by the inclusion therein of a minor proportion of an oil-soluble, phosphorus-bearing derivative of an organic hydroxy-acid which derivative is obtained from the reaction product of the acid with a phosphorus- and halogen-containing reagent of the type in which the phosphorus is trivalent.

6. A composition of matter comprising a major proportion of a liquid hydrocarbon having included in solution therein a minor proportion of a compound containing phosphorus in tri-

valent state, at least one bond of which is attached to the radicle  $-OR'COOR'$  where  $R$  is an organic radicle and  $R'$  is selected from the class consisting of an organic radicle, hydrogen, a metal and a metallic radicle.

7. A lubricating composition comprising a major proportion of mineral oil, the properties of which affecting its use as a lubricant in the crankcase of an internal combustion engine are improved by the inclusion therein of a minor proportion of the phosphorus-containing product resulting from the reaction of an ester of a mono-basic hydroxy acid with a phosphorus and halogen-containing compound of the type in which the phosphorus is present in tri-valent form.

8. A lubricating composition comprising a major proportion of mineral oil, the properties of which affecting its use as a lubricant in the crankcase of an internal combustion engine are improved by the inclusion therein of a minor proportion of the phosphorus-containing product resulting from the reaction of an ester of a saturated mono-basic hydroxy acid with a phosphorus and halogen-containing compound of the type in which the phosphorus is present in tri-valent form.

9. A lubricating composition comprising a major proportion of mineral oil, the properties of which affecting its use as a lubricant in the crankcase of an internal combustion engine are improved by the inclusion therein of a minor proportion of the phosphorus-containing product resulting from the reaction of an ester of a low molecular weight saturated mono-basic hydroxy acid with a phosphorus and halogen-containing compound of the type in which the phosphorus is present in tri-valent form.

10. A lubricating composition comprising a major proportion of mineral oil, the properties of which affecting its use as a lubricant in the crankcase of an internal combustion engine are improved by the inclusion therein of a minor proportion of the phosphorus-containing product resulting from the reaction of an ester of a low molecular weight saturated mono-basic hydroxy acid and a mono or di-hydric alcohol with a phosphorus and halogen-containing compound of the type in which the phosphorus is present in tri-valent form.

11. A lubricating composition comprising a major proportion of mineral oil, the properties of which affecting its use as a lubricant in the crankcase of an internal combustion engine are improved by the inclusion therein of a minor proportion of the phosphorus-containing product resulting from the reaction of an ester of a low molecular weight saturated mono-basic hydroxy acid and a low molecular weight mono or di-hydric alcohol with a phosphorus and halogen-containing compound of the type in which the phosphorus is present in tri-valent form.

12. A lubricating composition comprising a major proportion of mineral oil, the properties of which affecting its use as a lubricant in the crankcase of an internal combustion engine are improved by the inclusion therein of a minor proportion of the phosphorus-containing product resulting from the reaction of an ester of a low molecular weight saturated mono-basic hydroxy acid and a low molecular weight mono-hydric alcohol with a phosphorus and halogen-containing compound of the type in which the phosphorus is present in tri-valent form.

13. A lubricating composition comprising a

major proportion of mineral oil, the properties of which affecting its use as a lubricant in the crankcase of an internal combustion engine are improved by the inclusion therein of a minor proportion of the phosphorus-containing product resulting from the reaction of an ester of a poly-basic hydroxy acid with a phosphorus and halogen-containing compound of the type in which the phosphorus is present in tri-valent form.

14. A lubricating composition comprising a major proportion of mineral oil, the properties of which affecting its use as a lubricant in the crankcase of an internal combustion engine are improved by the inclusion therein of a minor proportion of the phosphorus-containing product resulting from the reaction of an ester of a saturated poly-basic hydroxy acid with a phosphorus and halogen-containing compound of the type in which the phosphorus is present in tri-valent form.

15. A lubricating composition comprising a major proportion of mineral oil, the properties of which affecting its use as a lubricant in the crankcase of an internal combustion engine are improved by the inclusion therein of a minor proportion of the phosphorus-containing product resulting from the reaction of an ester of a low molecular weight saturated poly-basic hydroxy acid with a phosphorus and halogen-containing compound of the type in which the phosphorus is present in tri-valent form.

16. A lubricating composition comprising a major proportion of mineral oil, the properties of which affecting its use as a lubricant in the crankcase of an internal combustion engine are improved by the inclusion therein of a minor proportion of the phosphorus-containing product resulting from the reaction of an ester of a low molecular weight saturated poly-basic hydroxy acid and a mono- or di-hydric alcohol with a phosphorus and halogen-containing compound of the type in which the phosphorus is present in tri-valent form.

17. A lubricating composition comprising a major proportion of mineral oil, the properties of which affecting its use as a lubricant in the crankcase of an internal combustion engine are improved by the inclusion therein of a minor proportion of the phosphorus-containing product resulting from the reaction of an ester of a low molecular weight saturated poly-basic hydroxy acid and a low molecular weight mono- or di-hydric alcohol with a phosphorus and halogen-containing compound of the type in which the phosphorus is present in tri-valent form.

18. A lubricating composition comprising a major proportion of mineral oil, the properties of which affecting its use as a lubricant in the crankcase of an internal combustion engine are improved by the inclusion therein of a minor proportion of the phosphorus-containing product resulting from the reaction of an ester of a low molecular weight saturated poly-basic hydroxy acid and a low molecular weight mono-

hydric alcohol with a phosphorus and halogen-containing compound of the type in which the phosphorus is present in tri-valent form.

19. A lubricating composition comprising a major proportion of mineral oil, the properties of which affecting its use as a lubricant are improved by the inclusion therein of from an effective amount to about 1% of an oil-soluble product resulting from the reaction of a hydroxy-ester with a phosphorus and halogen containing compound of the type in which the phosphorus is present in the tri-valent form.

20. A lubricating composition comprising a major proportion of mineral oil which has been stabilized by the inclusion therein of from about .001% to about .2% of an oil-soluble product resulting from the reaction of a hydroxy-ester with a phosphorus and halogen containing compound of the type in which the phosphorus is present in the tri-valent form.

21. A lubricating composition comprising a major proportion of a lubricating oil the resistance of which to oxidation is improved by the inclusion therein of from about .01% to about .1% of the product resulting from the reaction of a hydroxy-ester with a phosphorus and halogen containing compound of the type in which the phosphorus is present in tri-valent form.

22. A composition of matter comprising a major proportion of a liquid hydrocarbon having included in solution therein from an effective amount to about 1% of a compound containing phosphorus in tri-valent state, at least one bond of which is attached to the radicle —ORCOOR', where R is an organic radicle and R' is selected from the class consisting of an organic radicle, hydrogen, a metal and a metallic radicle.

23. A composition of matter comprising a major proportion of a liquid hydrocarbon which has been stabilized by the inclusion therein of from about .001% to about .2% of a compound containing phosphorus in tri-valent state, at least one bond of which is attached to the radicle —ORCOOR', where R is an organic radicle and R' is selected from the class consisting of an organic radicle, hydrogen, a metal and a metallic radicle.

24. A composition of matter comprising a major proportion of a liquid hydrocarbon, the resistance of which to oxidation has been improved by the inclusion in solution therein of from about .01% to about .1% of a compound containing phosphorus in tri-valent state, at least one bond of which is attached to the radicle —ORCOOR', where R is an organic radicle and R' is selected from the class consisting of an organic radicle, hydrogen, a metal and a metallic radicle.

CARL F. PRUTTON.  
ALBERT K. SMITH.  
DELTON R. FREY.